

Patented Nov. 28, 1950

2,532,155

## UNITED STATES PATENT OFFICE

2,532,155

## THIXOTROPIC INVESTMENT MATERIAL

Elbert E. Ensign, Ypsilanti, Mich., assignor to  
 Ford Motor Company, Dearborn, Mich., a corporation of Delaware

No Drawing. Application October 7, 1947,  
 Serial No. 778,469

4 Claims. (Cl. 22—188)

1

This application is concerned with the foundry molding art and more particularly with a process for the precision casting of metals by the investment or "lost wax" process. Basically this process depends upon the use of a destructible pattern constructed of wax, low melting point metal, combustible or soluble material. Such a pattern is surrounded or "invested" in a hardenable mixture which is then permitted to set or harden. The mold so prepared and containing the pattern is then treated to remove the pattern. If wax is chosen as the pattern material it can be removed by gentle heating to melt the wax. A similar treatment can be applied to low melting metal patterns. The combustible or soluble patterns can be removed by heating or dissolving. The choice of pattern material for any particular use is dictated by considerations well known to those skilled in the art and need not be elaborated upon here.

There are many satisfactory investment materials for the lower melting alloys and metals such as pewter, aluminum, bronze, brass, etc. However, attempts to extend the use of investment casting to steel have met with only limited success because of the lack of a really satisfactory investment material. Such a material must be strong and thermally stable to give a faithful reproduction of the original pattern. In addition, it must be sufficiently refractory to remain in contact with molten steel at temperatures circa 3000° F. without fusing or gassing and must under these high temperatures impart to the metal a smooth surface. In addition to the above, a commercially successful investment material must be fairly cheap if precision casting is to be competitive with other methods of fabrication.

To date the most widely used investment molds for use with steel have contained silica obtained from the hydrolysis of ethyl silicate or other organic ester of silicic acid. While such organo-silica compounds did yield satisfactory castings, they are objectionable commercially because of their cost. Applicant's endeavors to produce an economical investment material for use in the precision casting of steel have resulted in the instant invention.

Accordingly it is an object of this invention to provide an investment material which is satisfactory for use with ferrous metal or other high melting material.

It is a further object of this invention to provide an investment material for steel which is cheap and devoid of toxic constituents. Other objects will become apparent as the description proceeds.

5 To provide such an investment material for use in ferrous casting, applicant has taken advantage of the thixotropic properties of zeolitic materials, either natural or synthetic. When properly prepared these zeolitic investment materials have the property of remaining plastic indefinitely as long as they are kept agitated and the loss of moisture is prevented. Thus large batches of investment material may be prepared in advance and used as required.

10 While natural zeolitic materials may be used in the manufacture of applicant's investment material, considerations of economy, convenience and reproducibility of results dictate the use of the synthetic materials. Silica flour which is a form of very finely divided silica is the base material employed in the manufacture of the synthetic zeolite. To such silica flour is added water, an acid, a source of aluminum ions and a source of sodium and/or potassium ions. The following is a specific example of a method for preparing a successful investment material. A solution was prepared comprising:

|                          | Per cent |
|--------------------------|----------|
| 25 Water                 | 83.5     |
| Sodium Phosphate         | 6.6      |
| Potassium alum           | 3.4      |
| Hydrochloric Acid 22° Bé | 6.5      |

15 One part of this solution was mixed with three parts of fine silica flour and intensively agitated at room temperature. Under these conditions a reaction took place to yield a plastic, synthetic zeolite. The proportions given are by way of illustration only and represent only one of an endless series of mixtures which can be employed for the same purpose. For example, ordinary sodium chloride can be employed instead of the sodium phosphate. Apparently it is only essential that a source of acid, aluminum ions and sodium and/or potassium ions be added. However, the anions used should be selected with regard to their behavior during the firing and subsequent pouring of the mold.

20 The use of applicant's thixotropic zeolitic investment materials requires no variation from previously developed techniques based upon the use of organic silicates. The only precaution to be observed is the constant agitation of the zeolitic material to prevent setting. The unused zeolite should, of course, be protected from loss of moisture.

25 What is claimed is:

1. The process of preparing a thixotropic investment material comprising mixing by weight 83.5 parts of water, 6.6 parts of sodium phos-

phate, 3.4 parts of potassium alum, 6.5 parts of 22° Bé. hydrochloric acid, adding to the solution so formed three times its weight of fine silica flour, and intensively agitating the mix at room temperature.

2. The process of preparing thixotropic investment molding material comprising mixing an aqueous solution containing a soluble acid and a soluble aluminum compound and a soluble compound chosen from the group consisting of sodium and potassium compounds with sufficient silica flour to give a molding material of the desired consistency and intensively agitating the mix.

3. The process of preparing a thixotropic investment molding material comprising mixing an aqueous solution containing a soluble acid, a soluble aluminum compound and a soluble sodium compound with sufficient silica flour to give a molding material of the desired consistency.

4. The process of preparing a thixotropic investment molding material comprising mixing an aqueous solution containing a soluble acid, and soluble aluminum compound and a soluble potassium compound with sufficient silica flour to give a molding material of the desired consistency.

ELBERT E. ENSIGN.

#### REFERENCES CITED

The following references are of record in the file of this patent:

#### UNITED STATES PATENTS

| 5  | Number    | Name     | Date           |
|----|-----------|----------|----------------|
|    | 1,052,514 | Poulson  | Feb. 11, 1913  |
|    | 1,756,623 | Behrman  | Aug. 29, 1930  |
|    | 1,872,183 | Porter   | Aug. 16, 1932  |
| 10 | 1,889,007 | Wallace  | Nov. 29, 1932  |
|    | 2,193,346 | Ruddle   | Mar. 12, 1940  |
|    | 2,213,530 | Montero  | Sept. 3, 1940  |
|    | 2,233,701 | Grossman | Mar. 4, 1941   |
|    | 2,237,592 | Dunbeck  | Apr. 8, 1941   |
| 15 | 2,237,593 | Dunbeck  | Apr. 8, 1941   |
|    | 2,256,456 | Dietert  | Sept. 16, 1941 |

#### OTHER REFERENCES

- American Foundryman, April 1947, page 36.  
(Copy in Division 3.)  
Bentonite, Its Properties, Mining, Preparation and Utilization, Bureau of Mines Technical Paper 438, page 10.  
The Minerals of Bentonite and Related Clays and their Physical Properties, by C. S. Ross and Earl V. Shannon, pages 88-90.